

Dec. 13, 1938.

E. J. MARTIN

2,140,161

SULPHURIC ACID TREATMENT OF DEWAXED PETROLEUM STOCKS AT LOW TEMPERATURE

Filed Nov. 14, 1934



INVENTOR

Edward J. Martin

BY

Penrice, Davis, Marion and Edmunds

ATTORNEYS

## UNITED STATES PATENT OFFICE

2,140,161

## SULPHURIC ACID TREATMENT OF DE-WAXED PETROLEUM STOCKS AT LOW TEMPERATURE

Edward John Martin, East Chicago, Ind., assignor to Sinclair Refining Company, New York, N. Y., a corporation of Maine

Application November 14, 1934, Serial No. 752,927

9 Claims. (Cl. 196—40)

This invention relates to improvements in the manufacture of lubricating oils from wax bearing petroleum stocks. In referring to lubricating oils, reference is intended to petroleum oils, having a viscosity upwards of 70 seconds at 100° F. Saybolt Universal.

More particularly, the invention provides an operation comprising the sulphuric acid treatment of dewaxed petroleum stocks at low temperature. The invention makes possible the production, with good economy, of lubricating oils of good color and of low Conradson carbon content, the development of good acid efficiencies, and improvement of the product, particularly with respect to color, with minimum losses during the refining operation.

According to the present invention, the petroleum stock is dewaxed and the dewaxed oil is treated with sulphuric acid while maintaining a temperature not substantially exceeding 0° F. during acid addition and acid contact and during the subsequent separation of sludge formed as a consequence of the acid treatment. The acid treatment of the dewaxed oil, and the subsequent sludge separation, are with advantage carried out at temperatures as low as —10° F. or lower. A temperature not substantially exceeding 0° F., or better not substantially exceeding —10° F., is with advantage maintained during wax separation as well as acid addition, acid contact and sludge separation. A previously dewaxed oil, however, may be cooled to the temperature to be maintained during acid treatment and sludge separation immediately prior to acid addition.

The acid treatment and sludge separation, in the combined operation of the invention, are with advantage carried out in the presence of an admixed diluent, a naphtha or a liquefied normally gaseous hydrocarbon or mixture of hydrocarbons such as the so-called "liquid propane" fraction comprising about 70% of propane, for example. Naphthas boiling within a range approximating 200°—400° F., naphthas having a boiling range of 200°—300° F. or of 300°—400° F. for example, are useful in carrying out the invention. Such diluents are with advantage added to the oil prior to the dewaxing operation. While the manner in which the dewaxing operation is carried out is not essential to the invention, the dewaxing operation of the combined operation of the invention is with advantage carried out in the presence of an admixed diluent as in conventional practice. The diluted dewaxed oil may then be subjected directly to the low temperature acid treatment. The same or a different diluent may,

however, be admixed with the oil following the dewaxing operation and before the acid treatment

In one advantageous embodiment of the invention, the wax bearing stock is diluted with a "liquid propane" or its equivalent, this stock mixture is chilled by vaporization of a part of the admixed "liquid propane", the wax thus precipitated is separated from the remaining oil-diluent mixture, and the dewaxed diluted oil is then subjected to acid treatment followed by sludge separation, the low temperature maintained during acid treatment and sludge separation in accordance with the invention being established by the chilling first mentioned.

When the dewaxed and acid treated oil, after sludge separation, is to be treated with an absorbent earth as a finishing operation, the absorbent earth is with advantage added to the diluent oil immediately after sludge separation and the oil-earth-diluent mixture is with advantage heated but once both to activate the absorbent earth and to vaporize the remaining diluent from the lubricating oil product. Not only is an operating economy thus effected, but also any danger of impairing the quality of the product by heating the acid treated oil to effect separation of the diluent except in contact with the absorbent earth is thus avoided. Reference to addition of the absorbent earth to the diluted acid treated oil "immediately" after sludge separation is intended to refer to addition of the absorbent earth to the acid treated oil before the acid treated oil has attained any temperature at which degradation due to the remaining acid or acid reaction products is involved. The absorbent earth is with advantage added to the oil before its temperature has risen much above that at which sludge separation is effected.

It has hitherto been proposed to subject undewaxed petroleum stocks to acid treatment at low temperature. It has also been proposed to subject undewaxed petroleum stocks to acid treatment at high temperature followed by chilling to a low temperature at which sludge and wax are together to be separated from the oil. The presence of the wax during acid treatment impairs the acid efficiency. Also, the separation of wax and sludge together from the oil is subject to inherent difficulties in that wax crystals present interfere with the formation and separation of the sludge and the sludge present interferes with the separation of the wax. This invention is distinguished from such proposals in that, according to this invention, the stock subjected to

acid treatment has previously been dewaxed. The acid treatment as well as the sludge separation, moreover, are, according to this invention, effected at low temperature.

5 The invention will be further described in connection with the accompanying drawing which, as a flow diagram, illustrates a specific embodiment of the combined operation of the invention.

10 Referring to the drawing: The wax bearing stock to be treated is mixed with an appropriate diluent, naphtha or liquid propane, as indicated at 1. The diluted wax bearing stock is chilled to a temperature of 0° F. or -10° F. or -20° F. for example as indicated at 2. Precipitated wax is separated from the chilled diluted stock as indicated at 3. The cold diluted dewaxed stock is subjected to treatment with concentrated sulphuric acid as indicated at 4 and the resulting sludge is separated as indicated at 5. An absorbent earth is added to the cold diluted dewaxed and treated stock as indicated at 6. This stock-earth-diluent mixture is heated as indicated at 7, the vaporized diluent is separated as indicated at 8 and condensed or liquefied to be re-used as indicated at 1, and the spent earth is separated from the finished lubricating oil as indicated at 9. The low temperature established by the chilling indicated at 2 is, with advantage, maintained with a 20 minimum increase through the wax separation, the acid treatment and the sludge separation indicated at 3, 4 and 5. The acid treatment and sludge separation indicated at 4 and 5 may, however, be effected at temperature somewhat above 30 the temperature of wax separation.

35 The invention will be further illustrated by the following examples of specific operations embodying the invention:

A Pennsylvania long residuum having a gravity 40 of 26.0° Bé., a viscosity of 131 seconds at 210° F. Saybolt Universal, a pour test of 55° F. and a Conradson carbon content of 2.154% was dewaxed in the conventional manner to produce a dewaxed oil having a gravity of 24.3° Bé., a viscosity of 150 seconds at 210° F. Saybolt Universal, a pour test of -10° F., a Conradson carbon content of 2.645%. One portion of this dewaxed oil was diluted with 1.5 times its own volume of naphtha. This oil diluent mixture was treated with 40 pounds per barrel of 66° Bé. sulphuric acid and the resulting sludge separated while maintaining a temperature during acid addition, acid contact and sludge separation of -10° F. The acid treated oil-diluent mixture was heated to a temperature of 500° F. in admixture with 20% by weight of added Olmstead earth. The sludge loss on the dewaxed oil amounted to 13.6%. After separation of the diluent and spent earth, a lubricating oil product having a gravity of 25.5° Bé., a viscosity of 125 seconds at 210° F. Saybolt Universal, a pour test of -8° F., a Conradson carbon content of 1.218% and of good color was obtained. Another portion of this dewaxed oil was diluted with three times its own volume of liquid propane. 55 This oil diluent mixture was treated with 40 pounds per barrel of 66° Bé. sulphuric acid and the resulting sludge separated while maintaining a temperature during acid addition, acid contact and sludge separation of -10° F. The acid treated oil-diluent mixture was heated to a temperature of 500° F. in admixture with 20% by weight of added Olmstead earth. The sludge loss on the dewaxed oil amounted to 13.6%. After separation of the diluent and spent earth, a lubricating oil product having a gravity of 25.8° Bé., a

viscosity of 123.3 seconds at 210° F. Saybolt Universal, a pour test of -10° F., a Conradson carbon content of 1.132% and of good color was obtained.

With respect to economy, it is to be noted that although, in carrying out the invention, wax separation and sludge separation are separately effected, the burden of refrigeration is not required to be increased since the intervening acid treatment is also effected at a low temperature.

I claim:

1. In the manufacture of lubricating oils from wax-bearing petroleum stocks, the improvement which comprises dewaxing the oil, and thereafter treating the dewaxed oil with concentrated sulphuric acid and separating the resulting sludge while maintaining a temperature not substantially exceeding 0° F. during acid addition, acid contact and sludge separation.

2. In the manufacture of lubricating oils from wax-bearing petroleum stocks, the improvement which comprises dewaxing the oil, thereafter treating the dewaxed oil with concentrated sulphuric acid and separating the resulting sludge while maintaining a temperature not substantially exceeding 0° F. during wax separation, acid addition, acid contact and sludge separation.

3. In the manufacture of lubricating oils from wax-bearing petroleum stocks, the improvement which comprises diluting the oil, dewaxing the diluted oil, and thereafter treating the dewaxed diluted oil with concentrated sulphuric acid and separating the resulting sludge while maintaining a temperature not substantially exceeding 0° F. during acid addition, acid contact and sludge separation.

4. In the manufacture of lubricating oils from wax-bearing petroleum stocks, the improvement which comprises dewaxing the oil, and thereafter treating the dewaxed oil in admixture with a diluent with concentrated sulphuric acid and separating the resulting sludge while maintaining a temperature not substantially exceeding 0° F. during acid addition, acid contact and sludge separation.

5. In the manufacture of lubricating oils from wax-bearing petroleum stocks, the improvement which comprises dewaxing the oil, and thereafter treating the dewaxed oil with concentrated sulphuric acid and separating the resulting sludge while maintaining a temperature not substantially exceeding 0° F. during acid addition, acid contact and sludge separation, adding an absorbent earth to the acid treated oil immediately after sludge separation, heating the oil-earth mixture and thereafter separating the spent earth from the oil.

6. In the manufacture of lubricating oils from wax-bearing petroleum stocks, the improvement which comprises dewaxing the oil, and thereafter treating the dewaxed oil in admixture with a diluent with concentrated sulphuric acid and separating the resulting sludge while maintaining a temperature not substantially exceeding 0° F. during acid addition, acid contact and sludge separation, adding an absorbent earth to the diluted acid treated oil immediately after sludge separation, heating the oil-earth-diluent mixture and separating the diluent and the spent earth from the oil.

7. In the manufacture of lubricating oils from wax-bearing petroleum stocks, the improvement which comprises dewaxing the oil, and thereafter treating the dewaxed oil with concentrated sulphuric acid and separating the resulting sludge while maintaining a temperature not substan-

tially exceeding  $-10^{\circ}$  F. during acid addition, acid contact and sludge separation.

8. In the manufacture of lubricating oils from wax-bearing petroleum stocks, the improvement which comprises dewaxing the oil, treating the dewaxed oil with concentrated sulphuric acid and separating the resulting sludge while maintaining a temperature not substantially exceeding  $-10^{\circ}$  F. during wax separation, acid addition, acid contact and sludge separation.

9. In the manufacture of lubricating oils from wax-bearing petroleum stocks, the improvement which comprises dewaxing the oil, and thereafter treating the dewaxed oil in admixture with a diluent with concentrated sulphuric acid and separating the resulting sludge while maintaining a temperature not substantially exceeding  $-10^{\circ}$  F. during acid addition, acid contact and sludge separation. 5

EDWARD JOHN MARTIN. 10

CERTIFICATE OF CORRECTION.

Patent No. 2,140,161.

December 13, 1938.

EDWARD JOHN MARTIN.

It is hereby certified that error appears in the printed specification of the above numbered patent requiring correction as follows: Page 3, first column, line 5, claim 8, before "treating" insert the word thereafter; and that the said Letters Patent should be read with this correction therein that the same may conform to the record of the case in the Patent Office.

Signed and sealed this 24th day of January, A. D. 1939.

Henry Van Arsdale

(Seal)

Acting Commissioner of Patents.